

Dec. 11, 1945.

A. L. STONE

2,390,624

METHOD OF BUILDING UP TUBULAR JOINT MEMBERS

Original Filed Sept. 25, 1939 4 Sheets-Sheet 1



Fig. 1.



Fig. 2.



Fig. 3.



Fig. 4.

Inventor  
Albert L. Stone.

Barber & Scantling

Attorneys.

Dec. 11, 1945.

A. L. STONE

2,390,624

METHOD OF BUILDING UP TUBULAR JOINT MEMBERS

Original Filed Sept. 25, 1939 4 Sheets-Sheet 2



Fig. 5.



Fig. 6.

Inventor  
Albert L. Stone.

Bailey & Scantling

Attorneys

Dec. 11, 1945.

A. L. STONE

2,390,624

METHOD OF BUILDING UP TUBULAR JOINT MEMBERS

Original Filed Sept. 25, 1939 4 Sheets-Sheet 3



Fig. 7.



Fig. 8.



Fig. 10.



Fig. 9.

Inventor  
Albert L. Stone.

Barber & Scantling

Attorneys.

Dec. 11, 1945.

A. L. STONE

2,390,624

METHOD OF BUILDING UP TUBULAR JOINT MEMBERS

Original Filed Sept. 25, 1939 4 Sheets-Sheet 4

Fig. 11.



Fig. 12.



Fig. 13.



Fig. 14.



Inventor  
Albert L. Stone.

Barber & Scantling

Attorneys.

## UNITED STATES PATENT OFFICE

2,390,624

## METHOD OF BUILDING UP TUBULAR JOINT MEMBERS

Albert L. Stone, Palos Verdes Estates, Calif.

Original application September 25, 1939, Serial No. 296,452. Divided and this application October 7, 1941, Serial No. 413,962

8 Claims. (Cl. 29—148.2)

This invention relates to methods of building up tubular joint members and is more particularly concerned with such methods as applied to the building up of drill pipe tool joints for oil well strings.

While the invention is particularly adaptable to the reconditioning of worn joints, and the description is therefore mainly devoted to that aspect, its principles are adapted to the fabrication of new joints, as will later appear, and certain of the claims are inclusive of that aspect.

This application is a division of my copending application entitled Method of building up tubular joint members, filed September 25, 1939, Serial No. 296,452, now Patent No. 2,262,210, November 11, 1941.

Drill stem tool joints are tubular and include a body portion and a reduced diameter, externally threaded pin portion at one or both ends of the body portion. An annular shoulder extends transversely from the base of pin portion to the outer periphery of the body portion.

While the invention may be utilized to advantage in connection with any type of tool joint susceptible of the described method of reconditioning, repair and external reinforcement or protection, it is of particular advantageous application to tool joints of the general character set forth in Patent No. 1,932,427, issued to Frederick Stone on Well pipe joint, October 31, 1933. Therefore, I will describe the invention as applied to this particular type of tool joint, but this is not to be construed as limiting the invention, considered in its broader aspects.

In the joint thus chosen for illustrative purposes, an overhanging lip is formed on the end of the body portion adjacent the base of the pin portion, the lip defining, with the periphery of the pin base, a substantially V-shaped groove, one defining wall presenting a conical shoulder facing towards the free end of the pin. This shoulder is carefully machined to be in very accurately spaced relation with a shoulder formed at the free end of the pin portion and so it may form a fluid-tight seal with a mating shoulder on a complementary joint box. The significance of the shoulder accuracy and its position relative to other elements of the tool joint, is fully pointed out in the above mentioned patent.

Such tool joints are exposed to extremely severe service conditions, and, being operated in the presence of highly abrasive drilling mud, wear thin in a relatively short time, the external peripheral wear reducing, of course, the radial extent of the described conical shoulders. It is ob-

vious that this wear not only creates a final hazardous condition, but even before that critical condition is reached the shoulder wear (or its spread by reason of reduced backing-up material) may greatly decrease the fluid-holding efficiency of the joint.

It is therefore a general object of the present invention to provide means whereby such joints, after considerable wear, may be expeditiously and relatively cheaply reconditioned, thereby greatly increasing their useful life with full efficiency, the reconditioning being such that it in no way harmfully distorts or weakens the joint but on the contrary strengthens and reinforces it even to the point of giving it greater radial bulk and wear resistant qualities than possessed by the original joint.

In my copending application entitled Well pipe joints, Serial No. 225,362, filed August 17, 1938, now Patent No. 2,259,232, I have disclosed several reconditioning methods which have met with success. However, I have since found it necessary to concern myself more particularly with the problem of reforming the conical shoulders for it will be recognized that since these shoulders must mate with complementary shoulders on the box, must be accurately spaced with relation to other joint elements, and must take both fluid and mechanical pressural strains of a high order, the reconditioning must be of a nature which will permit the attainment of all these ends. It is therefore among the objects of the present invention to provide a reconditioning method which will fulfill all the required conditions, and yet do this without destroying the economic advantage of reconditioned joints. In other words, the end is attained by relatively rapid manufacturing steps and at relatively low cost.

Other objects and features of novelty of the invention will be made apparent in the following detailed description, reference being made to the accompanying drawings, in which:

Fig. 1 is a fragmentary sectional view through an unworn tool joint, showing in dotted lines how the wear may develop;

Figs. 2, 3 and 4 shows progressive steps in following this embodiment, Fig. 4 being an enlarged, fragmentary section of the welded shoulder in its final form as the result of the last step;

Figs. 5 and 6 show successive steps in a variational embodiment of the invention;

Figs. 7 to 10, inclusive, show successive steps in another variational embodiment of the invention;

Figs. 11 to 14, inclusive, show the adaptation of the invention to the fabrications of a new joint.

I will first describe Fig. 1 which, in full lines, represents one end of an unworn tool joint and, in dotted lines, shows how wear may occur. As said previously, the choice of this particular type of joint for illustrative purposes is not to be construed as limitative on the broader aspects of the invention, though the invention may be applied with particular advantage to this type of joint.

Ordinarily such tool joints are double-ended, and it will be understood that in such cases both ends may be treated in the manner here described as applying only to one end.

Tubular tool joint member 10, made, for instance, of steel, includes a relatively large diameter, cylindric body portion 11 and a relatively small-diameter pin portion 12. The pin portion has an external two-step thread 13, there being a tapered nose 14 at the free end of the pin portion, while there is an unthreaded and slightly tapered peripheral extent 15 at the base end of the pin portion. For purposes of clearer illustration, the taper of extent 15 is here shown exaggerated in degree.

Body portion 11 has an overhanging end lip 16 which, with peripheral extent 15 defines a substantially V-shaped groove 17, the lip face 18 presenting a conical shoulder facing towards the free end of the pin portion and tapering in a direction opposite that of nose 14. For reasons fully set forth in the aforementioned patent, shoulder 18 is very accurately spaced from nose 14 and is carefully machined so it may mate with the free end of a complementary box (not shown) to form a fluid tight joint. Lip 16 is also depended upon to hold the interfitting box end from diametral spread when the box and pin are subjected to longitudinal compressive strains by reason of the threaded joint between member 10 and the box being made up with predetermined tightness. It will thus be seen that shoulder 18 is a critical element of the joint, both as to its location and as to its formation. In connection with the latter aspect, it will be seen that any reformation of the shoulder during reconditioning operations must leave that shoulder so it will take with full efficiency the severe fluid and mechanical pressural strains to which it will later be exposed in use.

Dotted lines 19 indicate how member 10 may be worn down through peripheral wear, which, of course, correspondingly reduces the radial extent of shoulder 18. Usually, the wear is such that the body portion becomes eccentric or out-of-round. In the figures which follow, the first step of each variational embodiment has been indicated as involving a truing of the body portion with respect to the member-axis by a turning operation. The extent of turning will depend upon the condition of each given joint and, of course, in some instances this preliminary truing is not essential, and therefore the indication of an initial cut is not to be construed as limitative on the broader aspects of the invention.

In Fig. 2 the body portion 11 has been turned true and is, of course, of less diameter than the worn diameter 19 of Fig. 1. Peripheral extent 15, which is intended to seat tightly on a complementary box shoulder (not shown) is left undisturbed, the juncture of this extent with the turned-down body-face 20 being indicated at 21, junction-point 21 lying at a point corresponding with the bottom of groove 17 of the original joint member and

the substantially coincident point where the bottom of the reformed groove is to lie.

A sleeve or sheath 23 of wear resistant material, such as manganese steel, is fitted about body-face 20, the sleeve being pre-formed with apertures 24 to receive subsequent plug-welds. The end 25 of sleeve 23 projects over peripheral extent 15 of pin portion 12, a groove 26, defining the longitudinal extent of end 25, being cut annularly about the sleeve either before or after it is applied. In either event, the bottom of the groove is preferably located substantially directly over point 21. In some cases it is desirable to cut the groove clear through to the joint stock after the sleeve is applied but before the welding operation starts, the portion 25 being given sufficient area and tightness of fit with taper 15 to hold it, as a ring, on the joint after it has thus been severed from the body portion of the sleeve.

It will be seen that end 25 inclusively occupies the position previously occupied by lip 16.

The thickness of sleeve 23 is preferably such as to give an outside diameter which will restore the joint at least to its original diameter, though it is sometimes desirable to increase the sleeve thickness to an extent which will make the over-all diameter of the member even greater than that of the original joint and thus give added wear-taking material and further increase the useful life of the joint member. This latter is the condition illustrated in Fig. 2.

Sleeve 23 is then plug-welded at 31 or otherwise suitably bonded to the body portion of the joint member, and the bottom of groove 26 is melt-welded through, whereupon the groove, itself, is filled with weld material 32, the welding operation including sufficient melt-welding to cause weld-penetration into the body and pin portions and into the sleeve at opposite sides of the groove 26, all approximately to the extent indicated in Fig. 3, thus weld-integrating all said penetrated elements by the weld-zone W.

Groove 33 (Fig. 4) is then cut to correspond approximately with original groove 17 and with the conical shoulder 34 corresponding with original shoulder 18 and spaced properly with relation to nose 14. It will be seen that lip 35 may be partially made up of weld material and partially of the stock of sleeve 23 impregnated to greater or lesser extent by the weld material. Lip 35 is thus integrated by weld zone W with sleeve 23, body portion 11 and (at 36) with pin portion 12, the integration being such that groove 33 is bounded by an integrated surface which offers no opportunity for fluid leakage between the original stock and the welded-on material, nor for spreading failure when the joint is subsequently exposed to heavy fluid or mechanical pressural effects.

The top of lip 35 may be cut down to correspond with the outside diameter of original lip 16 and weld 32 then turned off as at 37 to merge that diameter into the outside diameter of sleeve 23.

In the description of the following variations, the same reference numerals will be given to parts which correspond to like elements in Figs. 1 to 4, without need of repeated individual description.

In the embodiment of Figs. 5 and 6, the method is generally the same as described in connection with Figs. 1 through 4, with the exception that, instead of utilizing a full-tube sleeve, there is here shown a sleeve or sheathing in the form of a spiral wrapping 23'. End 25' extends over pe-

peripheral extent 15 and is provided with a weld groove 26' located approximately over point 21. In this case, the sheathing is weld-integrated with the body portion of the joint by filling in the spaces between the spiral coils as at 50 (Fig. 6).

Groove 26' is welded through (Fig. 6) as described in connection with Fig. 3, a suitable dam D (Fig. 5) preferably being arranged at the outer junction of the spiraled groove and groove 26'.

The end-groove, overhanging lip and joint shoulder will then be formed in a manner similar to that previously described and illustrated in Fig. 4.

In Figs. 7 to 10, inclusive, another variation is shown. The first step is to fill groove 17 with weld material 55, preferably extending this "fill" over peripheral extent 15 even beyond the overhanging lip 16. Weld material 55 penetrates the lip, pin and body portions of the joint member as indicated in Fig. 7.

The body portion, lip and weld 55 are then turned down as indicated in Fig. 8, and a wear resistant sleeve 56 is fitted about the joint member as illustrated, the sleeve fitting the turned, peripheral face 57 of weld 55 as well as the turned face of the body portion.

Either before or after application of the sleeve, that sleeve is annularly grooved at 58, the groove being located substantially directly over point 27. The bottom of groove 58 is then melt-welded through and the groove filled with weld material 59, giving the general effect of Fig. 9, weld material 59 integrating the sleeve material at opposite sides of the original weld-groove, and, by virtue of its integration with weld material 55, integrating the sleeve material with the pin and body portions. Weld zone W thus includes integrated welds 55 and 59.

The end-groove, overhanging lip and joint shoulder are then formed (Fig. 10) in a manner similar to that previously described and illustrated in Fig. 4. The end of the lip may be chamfered as at 64, if desired.

If, desired, a second weld groove 60 may be provided in sleeve 56, adjacent groove 58, and when the bottom of this second weld-groove is welded through and the groove filled with weld-material 61, that material 61 additionally integrates the sleeve and body portion and, by virtue of the weld integration between material 59 and 61, there is a further tie between all the named elements.

Additional weld-groove 62 may be provided in sleeve 56 at a point longitudinally spaced from groove 61 and used for providing a melt-weld bond 63 between body portion 11 and sleeve 56.

In Figs. 11 to 14, inclusive, is shown an adaptation of the method to the fabrication of new joints. One of the distinct advantages gained by this adaptation, is the fact that it enables the use of relatively thin-walled tubing for the body portion of the joint, the extra stock for supplying the central enlargement, and the shoulders at the ends of that enlargement, being supplied by way of a sleeve which is weld-integrated with the body and pin portions. Obviously, this is of economic advantage over the usual custom of starting with tubing stock whose wall thickness is, throughout, that of the central enlargement and then cutting down the ends to the required reduced-diameter of the threaded pins. But in building up the stock with the sleeve and with the rigid requirements as to the shoulder characteristics, spoken of above, it will

be seen that this expedient calls for certain precautionary measures—measures which this invention supplies.

In Fig. 11, the operations start with a tube 70 whose normal thickness is represented at 71, which is considerably less than the final overall thickness the joint is to possess. Threads 13 and nose 14 are formed at one end of the tube, with extent 15' stopping short of the point 27' where shoulder 34" (Fig. 14) is ultimately to start. Sleeve 23", which may be chosen from a stock of sleeve of different thicknesses to suit the particular thickness-requirement of any given job, is then applied (Fig. 12) in the manner described in connection with Fig. 2, with groove 26' located over point 27'. The weld is then accomplished (Fig. 13) in the manner described in connection with Fig. 3, and the joint is finished off (Fig. 14) in the manner described in connection with Fig. 4 (except that the cut 37 need not necessarily be taken), with all the advantages described in connection with Fig. 4. An additional weld-bond between sleeve and tube may be provided at 63', as described in connection with Figs. 8 and 10.

While I have described preferred embodiments of my invention, it will be understood various changes may be made without departing from the spirit and scope of the appended claims.

I claim:

1. The method of reconditioning a tubular joint member that has a body portion, a reduced-diameter pin portion at one end of the body portion and an annular shoulder extending transversely of the joint member from the body portion to the pin portion and in predetermined longitudinally spaced relation with the free end of the pin, the reconditioning to include the re-forming of said shoulder; that includes turning down the body portion, fitting a sleeve to said turned-down body portion, with the end of the sleeve projecting beyond the end thereof over the pin portion adjacent the shoulder, forming an annular, peripheral groove in and spaced from one end of the sleeve and located approximately over the predetermined location of the re-formed shoulder, melt-welding through the groove bottom and weld integrating the sleeve at both sides of the groove with the joint member, substantially filling the groove with weld material and weld-integrating the material with the defining walls of the groove, and cutting an annular shoulder in the sleeve material and in the zone of weld in said predetermined spaced relation with the free end of the pin.

2. The method of reconditioning a tubular joint member that has a body portion, a reduced-diameter pin portion at one end of the body portion, and an overhanging lip on the body portion that defines with the base end of the pin portion an annular groove presenting a conical shoulder facing toward the free end of the pin; that includes filling said groove with weld material and weld-integrating the material with the defining walls of the groove to form an integrated fill-weld, flush-turning said body portion and fill-weld to true them with respect to the member axis, fitting a sleeve of wear-resistant material on the turned surface of the body portion and fill-weld, there being an annular weld-groove formed in the sleeve and spaced from one end thereof, locating said weld-groove over the bottom of the original shoulder-forming groove, melt-welding through the weld-groove bottom and thus weld-integrating the sleeve with the

joint member and fill-weld, substantially filling the original weld-groove with weld material and weld-integrating the material with the defining walls of said weld-groove, and cutting a groove in said sleeve material and in the zone of weld corresponding substantially to the shoulder-forming groove of the member in its original condition.

3. The method of reconditioning a tubular joint member that has a body portion, a reduced-diameter pin portion at one end of the body portion, and an overhanging lip on the body portion that defines with the base end of the pin portion an annular groove presenting a conical shoulder facing toward the free end of the pin; that includes filling said groove with weld material and weld-integrating the material with the defining walls of the groove to form an integrated fill-weld, flush-turning said body portion and fill-weld in true relation with respect to the member axis, fitting a sleeve of wear-resistant material on the turned surfaces of the body portion and fill-weld, there being an annular weld-groove formed in the sleeve and spaced from one end thereof, locating said weld-groove over the bottom of the original shoulder-forming groove, melt-welding through the weld-groove bottom and thus weld-integrating the sleeve with the joint member and fill-weld, substantially filling the weld-groove with weld material and weld-integrating the material with the defining walls of said weld-groove, there being a second annular weld-groove formed in the sleeve adjacent the first weld-groove, melt-welding through the bottom of the second weld-groove and through one side wall of the second weld-groove and into the weld material in the first mentioned weld-groove, and substantially filling said second weld-groove with weld material and weld-integrating the material with the defining walls of said second weld-groove, and cutting a groove in said sleeve material and in the zone of weld over the bottom of the original shoulder-forming groove and corresponding substantially to the shoulder-forming groove of the member in its original condition.

4. The method of reconditioning a tubular joint member that has a body portion, a reduced-diameter pin portion at one end of the body portion, and an overhanging lip on the body portion that defines with the base end of the pin portion an annular groove presenting a conical shoulder facing toward the free end of the pin; that includes filling said groove with weld material and weld-integrating the material with the defining walls of the groove to form an integrated fill weld, applying a sleeve to the body portion with its end projecting over the fill-weld, weld-integrating the end of the sleeve with said fill-weld, and cutting a groove in the zone of weld and corresponding substantially to the groove of the member in its original condition.

5. The method of reconditioning a tubular joint member that has a body portion, a reduced-diameter pin portion at one end of the body portion, and a shoulder extending between the portions and facing toward the free end of the pin; that includes building up by welding operations an annulus of weld material about the base end of the pin portion and integrated with the body

portion at the shoulder, applying a sleeve to the body portion with its end projecting over the weld-material annulus, weld-integrating the sleeve and annulus, and cutting a shoulder in the zone of weld and corresponding substantially to the shoulder of the member in its original condition.

6. The method of reconditioning a tubular joint member that has a body portion, a reduced-diameter pin portion at one end of the body portion and an annular shoulder extending transversely of the joint member from the body portion to the pin portion and in predetermined longitudinally spaced relation with the free end of the pin, the reconditioning to include the reforming of said shoulder, that includes turning down the body portion, cutting an annular, peripheral groove in a sleeve at a point spaced from one end thereof, fitting said sleeve to said turned-down body portion so said one end of the sleeve projects beyond the end of the body portion and over the pin portion adjacent the shoulder and so said groove overlies the predetermined location of the reformed shoulder, melt-welding through the groove bottom and weld-integrating the sleeve at both sides of the groove with the joint member, substantially filling the groove with weld material and weld-integrating the material with the defining walls of the groove, and cutting an annular shoulder in the sleeve material and in the zone of weld in said predetermined spaced relation with the free end of the pin.

7. The method of building up a tubular joint member, that includes tightly fitting an external sleeve to a tubular element, weld-integrating the sleeve and the tubular element with an annular weld extending radially through the sleeve from the outer periphery thereof and into the element, and in a zone which is axially inwardly spaced from both ends of the sleeve but is nearer to one sleeve-end than it is to the other, said weld extending continuously about the member in a plane normal to the longitudinal axis of the member, and cutting an annular shoulder in said annular weld with the shoulder extending transversely of the member axis and being exposed at said one end of the sleeve as an end seat for said joint member.

8. The method of building up a tubular joint member, that includes tightly fitting an external sleeve to a tubular element, weld-integrating the sleeve and the tubular element with an annular weld extending radially through the sleeve from the outer periphery thereof and into the element, and in a zone which is axially inwardly spaced from both ends of the sleeve but is nearer to one sleeve-end than it is to the other, said weld extending continuously about the member in a plane normal to the longitudinal axis of the member, cutting away a part, at least, of said one end of said sleeve where it extends axially beyond the weld and cutting away a portion of said annular weld to form in the sleeve and weld a continuous annular shoulder extending transversely of the member axis and being exposed at said one end of the sleeve as an end seat for said joint member.